

March 9, 1943.

R. A. DIMON

2,313,422

METHOD OF PICKLING METALLIC STRIP

Filed April 28, 1939



Inventor:

RICHARD A. DIMON,

by: *John E. Jackson*  
his Attorney.

## UNITED STATES PATENT OFFICE

2,313,422

## METHOD OF PICKLING METALLIC STRIP

Richard A. Dimon, Pittsburgh, Pa., assignor to  
Carnegie-Illinois Steel Corporation, a corpora-  
tion of New Jersey

Application April 28, 1939, Serial No. 270,703

1 Claim. (Cl. 204—145)

The present invention relates to a continuous method for the preparation of the surface of metallic strip.

In the coating of metallic surfaces, especially in the electroplating thereof, it is well recognized that the properties of the resulting coating, in particular its adherence to the base metal, are greatly influenced by the conditioning treatments given the metallic surface prior to the coating operation. In the case of certain electrodeposited metallic coatings, for example tin, it is known that the base metal must be micro-roughened to a definite degree if a tightly adherent tin coating is to be obtained. In the past such roughening of the surface has been generally obtained by pickling the metallic material in an acid solution, sufficient time being allowed for the acid not only to remove any oxide present but to actually chemically attack (etch) the surface to the desired degree. The time required in such a pickling step is of the order of a minute or two. In the plating of sheets or irregular shaped objects which operations are themselves slow, such a length of pickling time has not been objectionable. However, in the continuous plating of metallic strip, it has proved a serious handicap since the economic operation of the latter process requires the utilization of high processing speeds.

It is apparent that the necessary pickling time could be obtained in a high speed continuous strip plating operation by increasing the size of the acid solution container. Such increase in size, however, not only adds to the cost of the equipment but requires considerable floor space which is itself valuable, and may not always be available.

While the use of an anodic pickling step would satisfy the time and space requirements of a high speed continuous strip operation, it has been experienced that such a step requires an excessive amount of control to avoid overpickling of the surface of the strip. Said overpickling results in a coated product having poor appearance.

The danger of overpickling is especially prevalent in a process which slows down the strip to join incoming and outgoing ends.

Under the present method, the aforementioned disadvantages are overcome.

An object of the present invention resides in providing an initial concentrated electrochemical pickling action at the surface of the continuously moving metallic strip and immediately thereafter continuing the pickling while in the same

pickling solution but in a purely chemical manner.

Other objects and advantages will become apparent as the description proceeds and reference is had to the accompanying drawing, in which:

The figure is a sectional elevation of the present invention.

The single figure of the drawing is a diagrammatic showing of a pickling tank and the manner in which the present invention is practiced therewith.

In the drawing, the metallic strip S is continuously fed over a conductor roll 3 into the pickling tank 2. Immediately at its point of entry into the pickling tank, the metallic strip is passed between two cathodes 4 which are connected to the negative side of a generator 5. The conductor roll 3 over which the incoming continuous metallic strip passes is connected to the positive side of the generator so as to establish the metallic strip as the anode, whereby as it passes between the cathodes 4 positioned at the entrance end of the pickling tank 2, the strip is immediately subjected to a violent electrochemical pickling action. This initial violent pickling of the metallic strip produces an active surface thereon which expedites the straight chemical action of the pickling solution on said surface during its passage through the remaining portion of the pickling bath.

The strip S, comprising base metal for tin plate or the like, is moved in a substantially vertical loop having the horizontal extent thereof, as by reason of the sinker roll shown in the drawing, relatively smaller or less than the vertical extent of said loop, whereby the pickling process may be effected within a minimum space in the direction of travel of the strip.

As a result of the initial vigorous electro-pickling action, underpickling, as would result were the material subjected to straight chemical action for the same time and in equipment of the same size, is avoided. Sufficient anodic pickling is thus given the strip so as to permit the chemical action of the acid in the succeeding portions of the tank to rapidly progress, whereby the high degree of control necessary to avoid overpickling as would be the case with anodic pickling alone, is eliminated.

The pickling bath may comprise a five per cent sulphuric acid solution maintained substantially at room temperature, the electrochemical step being carried out at a current density of 100 amperes per square foot. Heating of the pickling solution which in the past has been gener-

ally recommended to obtain the best results is not necessary since, under the present invention, the surface of the metallic strip is rapidly initiated by the initial electrochemical action. Solutions other than sulphuric acid may be used, such for example, a five per cent solution of hydrochloric acid or any other desirable pickling solution.

By such a method, equipment can be used requiring a minimum amount of floor space and, at the same time, provides for the time factor which is important in the high speed continuous treatment of metallic strip being fed into and out of the pickling bath.

While I have shown and described a specific embodiment of the present invention, it will be seen that I do not wish to be limited exactly thereto, since various modifications may be made without departing from the scope of the invention, as defined by the following claim.

I claim:

The method of continuously pickling base

metal strip for tin plate and the like, which includes moving the said strip in a substantially vertical loop through an effective pickling solution, said loop being characterized by having the horizontal extent thereof relatively smaller than its vertical extent, imparting to the strip a violent anodic pickling action at the immediate point of its entry into the said pickling solution, continuing the violent anodic pickling action for only a portion of the length of downward vertical travel of the strip through the pickling solution, and discontinuing the violent anodic pickling action at a substantial distance from the end of the length of downward travel of the strip, the remainder of the length of travel of the strip being conducted through the pickling solution while subjected to a pickling action which is entirely chemical, the said anodic and chemical pickling comprising the only pickling to which the strip is subjected in said solution.

RICHARD A. DIMON.